

## UNITED STATES PATENT OFFICE.

LOUIS F. CLARK, OF GRAND RAPIDS, MICHIGAN, ASSIGNOR TO UNION CARBIDE SALES COMPANY, OF NEW YORK, N. Y., A CORPORATION OF WEST VIRGINIA.

## TREATMENT OF COPPER MINERALS.

No Drawing.

Application filed October 29, 1923. Serial No. 671,392.

The invention is a process for recovering the values of ores by flotation concentration. It is applicable where the metal ultimately to be produced is copper, silver, or mercury, 5 and is particularly useful for the treatment of certain copper ores.

The sulphide minerals of copper, such as chalcocite and chalcopyrite, are usually readily amenable to flotation concentration. The 10 oxide minerals, such as cuprite, and the carbonate minerals, such as malachite, can not be readily floated, and this is also true of native copper. Even ores wherein the copper exists predominantly in combination 15 with sulphur sometimes give poor recoveries when flotation is applied to them. This may be due to superficial oxidation, or to less understood causes connected with the nature of the minerals with which the sulphite is 20 associated in the ore. The process to be described gives increased amenability to flotation when applied to many copper minerals and particularly to those which are not 25 adapted for flotation concentration by standard methods.

Copper minerals in an ore may be so closely associated, either by chemical combination or physical proximity, with the minerals of other metals, that a process intended to make a copper mineral floatable 30 may also aid in the flotation of the other minerals. But if such close association does not exist it is possible by a proper use of my invention to select only the copper minerals 35 in the ore and to separate them from the other minerals.

Copper minerals may be classified as "cupric" and "cuprous" depending on the state of oxidation of the element. Both 40 these classes are amenable to the treatment herein described.

I have found that cupric copper in alkaline, neutral or slightly acid solution, in the presence of acetylene, becomes an oxidizing agent because of its tendency to precipitate 45 as a cuprous compound, cuprous acetylide. In order to produce this effect an oxidizable compound must also be present. This oxidizable compound may be acetylene itself, 50 or some other oxidizable substance either organic or inorganic, for example carbon monoxide or glucose. In some cases it is advantageous to use an oxidizable substance which can be converted into an insoluble

compound, such as a resin, by oxidation. 55 Examples of this class of compounds are aniline, linseed oil, turpentine, and pine oil. Under suitable conditions the insoluble organic oxidation product is precipitated with 60 the cuprous acetylide.

I have applied the above principle to the treatment of copper minerals, especially the oxide minerals, in an ore pulp. Such copper minerals, in a water pulp in the presence of dissolved acetylene, are able to oxidize at 65 their surface any oxidizable compound simultaneously dissolved. Thus a coating takes place on the surface of the copper mineral, primarily of the compound cuprous acetylide. If for example aniline, or turpentine, are also present dissolved in the water, then a composite coating is produced whose second component is the insoluble oxidation product of such organic substance, 70 or the organic resin. It is a coating of this 75 nature which seems to be especially favorable to subsequent flotation of the coated minerals.

The conditions under which this principle may be applied are variable and may 80 be adjusted to produce different degrees of the coating effect. The principal items for consideration are the following:—

(a). The hydrogen ion concentration of the water used to make up the pulp, together 85 with the influence of dissolved salts. This determines the extent to which the copper minerals may be superficially attacked so as to render them more amenable to the coating reaction and it also influences the rapidity of the coating reaction itself. Thus, slightly acid pulps may be desirable with some ores. "Slightly acid" is here intended generally to express an acidity caused by the hydrolysis of a weak-base salt, e. g. 90 ferrous sulphate. Free sulphuric acid might also be present in traces, but although it might help to attack the minerals, it might delay the required coating action and eventually might prevent it entirely. This is 100 because the coating reaction itself makes acid by hydration and oxidation of the acetylene to acetic acid. On the other hand alkaline pulps may be desirable. The alkalinity may be brought about by addition 105 of lime or soda ash or caustic soda. Frequently also addition of ammonia is helpful. These reagents tend to film the copper

silicates and other compounds with copper hydroxide which is itself especially adaptable to the coating reaction. Again, a combination of these conditions may be useful, 5 as, for example, a treatment first with a weak solution of ferrous sulphate or sulphuric acid, followed by addition of alkali and the coating reagents. Also, the addition of other reagents may be useful for both 10 purposes, e. g. sodium silicate, phosphate, chloride and so forth.

(b). The temperature of the solutions together with the concentration of the various substances dissolved are important. In 15 general, especially if an alkaline pulp is used, a warm solution is better than a cold one. Particularly it might be advantageous to heat an alkaline pulp during the operation of grinding so as to increase the formation 20 of hydroxide on the surfaces of the mineral particles. On the other hand, warming the pulp decreases the solubility of the most important element of the coating reagents, viz, the acetylene. Thus if a warm pulp is 25 used it may be necessary to enclose it and inject acetylene gas under pressure.

(c). The time during which the reagents are allowed to act upon the mineral particles is also important. Both the action of 30 the surface attack on the mineral particles and the coating effect itself, are rather slow in operation. Warming the pulp seems to reduce the time required.

The preceding paragraphs have spoken 35 perhaps too definitely of two phases of the procedure; first the attack on the surfaces of the mineral particles, and then the coating effect. In reality in operation it would be difficult to say when one of these took 40 place and the other began or to tell their comparative extent. Similarly the whole coating result on one mineral might be quite different from that on another, and yet both give good flotation. In one case a coating 45 very heavy and black might be required and in other an effect not visible to the naked eye would be sufficient for satisfactory flotation.

It should also be noted that this coating 50 by the action of acetylene implies the injection and dissolution of the gas in the liquid of the pulp. After sufficient action has taken place the excess gas may be removed from solution by heating the pulp 55 or applying a vacuum.

This process of coating the copper minerals in an ore pulp for flotation concentration may in general be applied with the regular machinery now in use for such ore 60 dressing.

An ore may be ground with a cold solution 65 of lime, ammonia, pine oil, a flotation oiling oil and acetylene gas. After grinding such a pulp might well be partially dehydrated or "thickened" to re-

duce the proportion of the liquid to the solid, say from a 4 to 1 to a 1 to 1 ratio. The recovered liquid would then be available as recovered water and recovered valuable and unused reagents to return to fresh 70 charges of ore. Such thickening operation would delay the advance of the solids and so increase considerably the time available for the coating operation to reach a satisfactory condition. Such a thickened pulp 75 would then be diluted with other water for the flotation operation.

An ore may be ground with a warm solution of caustic soda, ammonia, glucose and a flotation oiling oil. The warm 1 to 1 pulp 80 may be collected in a container and then acetylene gas injected so that the whole is under pressure. The pulp should then be diluted with cold water and classified. Particles which had not been finely ground in 85 the first instance would then come through again for further coating.

An ore may be ground with a cold solution of ferrous sulphate, aniline, acetylene and a flotation oiling oil. Later in its progress 90 such a pulp may, or not, be made alkaline, say with lime and the flotation operation carried out. The tail pulp from such an operation should be settled to recover valuable solution for reuse on fresh charges 95 of ore.

In any or all of these cases the flotation oils may be omitted or applied at other points in the scheme of operation. Likewise the injection of the acetylene to form 100 a solution of the gas in the pulp may be effected at any convenient point and by suitable means, as for example blowing the gas into the liquid through a porous diaphragm in order to diffuse it into the liquid in the 105 form of very fine bubbles.

In an example of the operation of this process the following may be considered; laboratory apparatus was used; 1200 grams of 20-mesh ore was ground in a ball mill 110 30 minutes with 1200 grams of water. The product of this gave about 75% of the mineral through a 200-mesh screen. The water also carried NaOH, 1 pound per ton of ore, and NH<sub>3</sub>, 0.80 pounds per ton. Temperature of pulp during grinding was 50° C. After grinding, the mixture was transferred to an autoclave using 1200 grams more of water as a wash, thus giving a 2 to 1 pulp. Now 1 pound more of NaOH per ton of ore 115 and 0.80 pounds more of NH<sub>3</sub> were added, together with two pounds per ton of ore of aniline oil. Acetylene gas was now injected while the pulp was agitated and held at about 50° C. A pressure of about 25 120 pounds per square inch was maintained. At the end of about 15 minutes the coating operation was completed and the excess gas blown off. The pulp was now diluted with cold water to a 5 to 1 ratio and flotation

125

conducted in a mechanically agitated machine using coal tar, creosote and pine oil. The following results were obtained.

Feed—2.10% total copper.

Feed—2.00% oxide copper.

Concentrate—14.50% total copper.

Concentrate—11.30% oxide copper.

Tails—0.77% total copper.

Tails—0.73% oxide copper.

Recovery on total copper, 65.40 per cent. This example indicates what might be expected when comparatively large amounts of the reagents are applied in warm solution for a short time. On large scale work and where operation might be made continuous in such an apparatus as has been mentioned wherein the gas may be injected and recovered from the pulp as it passes through a pressure container, more thorough coating may be expected and accordingly better flotation results.

In another example 1200 grams of 20-mesh ore were ground 30 minutes with 1200 grams of water which contained 0.80 pounds of  $\text{NH}_3$  and 1 pound of  $\text{NaOH}$  per ton of ore. A temperature of  $50^\circ \text{ C}$ . was maintained during grinding. After grinding, the pulp was cooled to about  $15^\circ \text{ C}$ . and 1200 grams of cold water added. This last water carried aniline oil and acetylene dissolved amounting to 1 pound of each per ton of ore. The pulp was agitated and then allowed to stand in the liquid for 24 hours. It was then diluted and flotation carried out as before noted. The following results were obtained.

Feed—2.09% total copper.

2.00% oxide copper.

Concentrate—20.90% total copper.

18.70% oxide copper.

Tails—0.79% total copper.

0.73% oxide copper.

Recovering on total copper, 62.00 per cent. This example illustrates the use of lesser amounts of reagents in cold solution where the coating action was allowed to proceed through considerable time. This indicates also the application before mentioned of a thickening device which would at once recover excess solution from the pulp and delay the advance of the solids until sufficient coating action had taken place.

This principle may be extended to a system of tank storage of thickened pulp containing small amounts of the required reagents dissolved. Coating action may be thus carried out over periods of days without reducing the tonnage capacity of the milling plant. In such a case, however, and especially where an alkaline solution is used. the pulp had best be protected as much as possible from sun light and air which would tend to cause consumption of acetylene by

oxidation to acetate. Aside from such slight action as this however, there should be no other chemical consumption of acetylene except on the surfaces of the minerals it is desired to coat. This is itself an important difference between the coating action of acetylene and of hydrogen sulphide. The latter coats indiscriminately iron, lead, copper and so forth and is thus largely consumed by worthless minerals.

Where the ores contain minerals of other metals than copper, most commonly iron, lead and zinc, the treatment described has a selective action. It acts only on the particles of the copper minerals present so that in the subsequent flotation it is only, or mainly the copper minerals which will be floated; so that the latter only will be selected and separated from other metals.

For the flotation operation to which the treated ore is subsequently subjected, any usual or suitable flotation oils and methods may be applied.

The treatment may be used also to recover by flotation other elements which may be closely associated with the copper minerals where the floatability of the particles is sufficiently great to carry the percentage of the other elements present in the particles. Where the ore contains mixed oxides and sulphides of copper it may be subjected first to a flotation operation on the pulp to remove the sulphides of copper (or in fact any other minerals which are naturally floatable) after which the present process may be applied to the residue carrying oxides of copper or other difficultly floatable copper-bearing constituents so as to make these suitable in a second operation.

There are ores of other metals than copper to which the invention may be applied. For example silver and mercury have great affinity for acetylene and the minerals of these metals may also be filmed with the acetylide and thus their flotation facilitated.

Though I have described with great particularity of detail certain embodiments of my invention, yet it is not to be understood therefrom that the invention is restricted to the particular embodiments described. Various modifications in the steps of the process and in their order and in the proportions of the ingredients stated may be made by those skilled in the art without departing from the invention as defined in the following claims.

What I claim is:—

1. The method of treating ores containing copper minerals to increase their susceptibility to flotation concentration by processes dependent upon affinity between minerals and a gaseous agent which consists in applying to a pulp of the ores acetylene and other oxidizable substances, the oxidation of which results in insoluble substances thus

producing on the particles of the said minerals a coating of cuprous acetylide and of the said insoluble oxidation products.

2. The method of preliminarily treating 5 ores containing copper minerals to increase their susceptibility to subsequent flotation concentration by processes dependent upon affinity between minerals and a gaseous agent which consists in applying to the particles thereof a coating containing cuprous acetylide.

3. The method of preliminarily treating 15 ores containing copper minerals to increase their susceptibility to subsequent flotation concentration by processes dependent upon affinity between minerals and a gaseous agent which consists in applying to a pulp of the ores acetylene gas under pressure, the temperature of the pulp being too high 20 to retain a substantial quantity of gas at atmospheric pressure.

4. The process which comprises treating a copper ore with acetylene until the floatability of the copper mineral is materially increased, and then floating the mineral, by 25 froth flotation.

5. The process which comprises treating a pulp of copper ore with acetylene until the floatability of the copper mineral is materially increased, and then floating the mineral, by 30 froth flotation.

6. In a process of concentrating copper ores, the step of treating a pulp of the ore with acetylene until the floatability of the copper mineral by processes dependent upon 35 affinity between minerals and a gaseous agent is materially increased.

7. The process which comprises rendering a pulp of copper ore alkaline; adding a non-gaseous reducing agent; treating the pulp 40 with acetylene until the floatability of the copper mineral is materially increased, and then floating the mineral, by froth flotation.

8. The process which comprises rendering a pulp of copper ore alkaline; adding an 45 organic reducing agent adapted to form a water-insoluble oxidation product; and treating the pulp with acetylene until the floatability of the copper mineral by processes dependent upon affinity between minerals and a gaseous agent is materially increased.

9. The process which comprises rendering a pulp of copper ore alkaline; adding aniline; treating the pulp with acetylene until the floatability of the copper mineral is materially increased, and then floating the mineral, by 55 froth flotation.

In witness whereof, I have hereunto signed my name.

LOUIS F. CLARK.